

## UNITED STATES PATENT OFFICE

2,068,919

PROCESS FOR THE PRODUCTION OF  
SOUND RECORDS

Gustav Kögel, Baden-Baden, Germany

No Drawing. Application March 27, 1936, Serial  
No. 71,336. In Germany November 24, 1934

15 Claims. (Cl. 274—46)

The present invention relates to a process for the production of sound records by mechanical means, such as are employed, for example, in gramophone records, in telegraphing photographs, in television and for similar purposes.

An object of the invention is a process for producing sound records on supports which consist of mixtures of glue, gelatine or similar colloids capable of being tanned and such light sensitive organic compounds as acquire under the influence of light tanning properties with regard to the colloids employed, but in the dark are inert with regard to the said colloids. The term "tanning" is employed in this specification to mean, as is universally customary, the diminution of the capability of taking up moisture or of the solubility of the colloids in moistening or solvent means respectively.

The supports described are provided in the customary manner by engraving, incising or by similar mechanical treatment with relief-like records, whereupon the records are fixed by simple exposure to light. By this exposure to light, in addition to the solubility and capability of being moistened the mechanical properties of the material are also altered in a surprising manner so that the material can be exceptionally well employed for the direct reproduction of sound. The lasting properties of the records and their resistance to injuries are also very good. Other objects of the invention are materials bearing sound records.

As light sensitive compounds higher molecular diazo compounds, particularly such as contain at least three carbocyclic rings, for example six rings, are suitable for use. Moreover, light sensitive carbonyl compounds, particularly quinones, may also be employed. Preferably the sulphonic acids of these compounds are used. Light sensitive dyestuffs, particularly light sensitive dyestuffs of an acid nature, for example xanthone dyestuffs, are also suitable for use. Furthermore many aromatic nitro compounds are suitable for use. As sensitizing agents the most varied nitro derivatives of the benzene and naphthalene series may, for example, be employed, particularly compounds of  $\alpha$ -nitro-naphthalene. Such compounds as are substituted by oxyalkyl groups or by acid groups, such as, for example, sulpho- or carboxyl groups, for example the  $\alpha$ -nitro-naphthalene derivatives which are substituted in the neighbouring position, i. e. in the peri- or ortho-position to the nitro group, come particularly into consideration. If water soluble colloids are used, such nitro compounds as are likewise soluble in water, such as, for example, 1-nitronaphthalene-8-sulphonic acid, 1-nitro-naphthalene-2-sulphonic acid, 1-nitro-naphthalene-8-carboxylic acid, 1-nitro-naphthalene-3,8-disulphonic acid, 1-nitro-8-methyl-naphthalene-4-sulphonic acid,

and which may possess still further substituents (such as, for example, halogens) may be employed. If colloids soluble in alcohol or hydrocarbons are used, 1-methyl-8-nitro-naphthalene and 1-nitro-naphthalene-8-carboxylic acid come, 5 for example, into consideration. Furthermore light sensitive dyestuffs, particularly xanthone dyestuffs, may be employed as sensitizing agents. In order to attain the best possible evaluation of the sources of light just according to their spectroscopic constitution, mixtures of various light sensitive substances may be employed if desired.

As colloids capable of being tanned there may be employed, besides the gelatinous substances coming into consideration in the first place, also 15 other albuminous substances, such as casein, furthermore collodion, asphalt, certain artificial resins, such as vinyl resins, and other substances. In known manner these substances may also be incorporated with materials such as graphite or 20 metal dust. The mixtures of the colloids with the light sensitive substances and the other additions are preferably dissolved in a solvent, for example, water, and are applied to suitable bases, for example metal plates, cardboard and so forth. 25 If desired, the supports may be already pre-exposed before the working operation in order to alter the degree of hardness of the material; in this manner the degrees of hardness which always vary with different gelatine preparations 30 can be equalized or compensated.

If desired the colloids capable of being tanned may be employed in admixture with waxes. In this manner supports are obtained, which can be sufficiently hardened by light and the particular advantage is further obtained that the adaptability for the mechanical working operation, particularly the adaptability for incising is better. By varying the quantity of wax it is possible to cause, as desired, either the adaptability for the working operation or the capability of hardening to predominate. In order to obtain a suitable pouring solution it is necessary in this case to mix the colloid capable of being tanned and the wax with one another in a solvent which is adapted for association with the two materials or does form permanent dispersions with the two materials respectively. In the case where gelatine is employed as the colloid capable of being tanned and bees' wax is employed as the wax, glycerine may, for example, be used as the solvent. Glycol may also be advantageously employed.

The following examples illustrate the invention:

(1) 1 litre of a 5% gelatine solution is mixed with 5 grams of eosine and 15 grams of thiosinamine, the mass obtained is cast into plates and dried. After the audition which is effected in known manner the plates are finished by expo- 60

sure to the light of an arc lamp for a period of, for example, a few minutes.

In place of the eosine, homologues, such, for example, as erythosine, rose bengale, phloxine, 5 cyanosine and others may be employed.

(2) A solution of 100 grams of gelatine in 500 c. c. of water is mixed with a solution of 20 grams of the magnesium salt of 1-nitro-naphthalene-8-sulphonic acid in 300 c. c. of water. With the 10 product thus obtained aluminium plates are coated, which are provided in the customary manner with sound records and are then exposed to light. In place of the magnesium salt of 1-nitro-naphthalene-8-sulphonic acid the following 15 pounds may also be employed: 1,2-nitronaphthalenesulphonic acid, 1,3,8-nitro-naphthalenedisulphonic acid, ortho-nitrobenzylalcohol, the sodium salt of 4-nitronaphthalene-1,8-dicarboxylic acid, the sodium salt of 1-nitronaphthalene-8-carboxylic acid. A further mixture which is suitable for 20 use for the production of supports of sound records consists of: 12 grams of the sodium salt of o-nitro-cinamimic acid, 140 grams of gelatine and 1000 c. c. of water.

(3) The procedure is carried out as in Example 25 2 but with the difference that instead of the gelatine solution mentioned in the said example casein plates or plates of agar-agar or albumins are employed as the starting material and the 30 said plates are impregnated with the solutions of a light sensitive substance specified in Example 2.

(4) 100 grams of gelatine powder are mixed with 60 c. c. of glycerine and the mass is melted together in the water bath. After the addition 35 of 20 grams of the magnesium salt of 1-nitro-naphthalene-8-sulphonic acid, 50 grams of bees' wax are stirred in. A very fine emulsion is thereby obtained which is cast into plates. The working-up is carried out according to Example 1. 40 Instead of the bees' wax it is also possible to employ, for example, Carnauba wax or Montan wax.

(5) 8 gram of o-nitrophenylpropionic acid and 100 grams of gelatine are dissolved in 1000 c. c. 45 of water. The mixture is worked up according to Example 1.

(6) 3 grams of a phenanthrenequinonesulphonic acid, preferably a disulphonic acid, for example 2,7-phenanthrenequinone-disulphonic acid 50 are dissolved together with 10 grams of gelatine in 120 c. c. of water and are cast into plates which are worked up according to Example 1. In place of the phenanthrenequinonesulphonic acids the corresponding derivatives of pyroanthraquinone may be employed.

(7) A mixture of 100 grams of gelatine, 8 grams of the zinc chloride compound of diazotized 4-amino-1(N-methyl-6-naphthalenetetrahydride-1, 2, 3, 4)-aminobenzene, 20 grams of 55 50% acetic acid and 800 cc of water is applied to celluloid film. The strips are provided with records by mechanical means and are finished by exposure to light under a quartz lamp.

I claim:

60 1. A process for the production of sound records, which comprises mechanically producing records on supports comprising in a mixture colloids capable of being tanned and such light sensitive organic compounds as exert a tanning action in the light on the said colloids, and fixing the records by exposure to light.

65 2. A process for the production of sound records, which comprises engraving records on sup-

ports comprising in a mixture colloids capable of being tanned and such light sensitive organic compounds as exert a tanning action in the light on the said colloids, and fixing the records by exposure to light.

5

3. A process for the production of sound records, which comprises engraving records on supports comprising in a mixture colloids capable of being tanned and light sensitive dyestuffs, and fixing the record by exposure to light.

10

4. A process for the production of sound records, which comprises engraving records on supports comprising in a mixture colloids capable of being tanned and light sensitive xanthone dyestuffs, and fixing the record by exposure to light.

15

5. A process for the production of sound records, which comprises engraving records on supports comprising in a mixture colloids capable of being tanned and high molecular diazo compounds which contain at least three carbocyclic rings, and fixing the record by exposure to light.

20

6. A process for the production of sound records, which comprises engraving records on supports comprising in a mixture colloids capable of being tanned and light sensitive nitro compounds, and fixing the record by exposure to light.

25

7. A process for the production of sound records, which comprises engraving records on supports comprising in a mixture colloids capable of being tanned and  $\alpha$ -nitro-naphthalene sulphonic acids, and fixing the record by exposure to light.

30

8. A process for the production of sound records, which comprises engraving records on layers comprising colloids capable of being tanned and such light sensitive organic compounds as exert a tanning action in the light on the said colloids, the said layers being supported by a base, and fixing the record by exposure to light.

35

9. The process which comprises engraving records on supports comprising colloids capable of being tanned and such light sensitive organic compounds as exert a tanning action in the light on the said colloids.

40

10. A phonograph record bearing engraved sound tracks, said record comprising a tanned colloid and the light decomposition product of such a light-sensitive organic compound as exerts a tanning action in the light on the un-tanned colloid.

45

11. A phonograph record bearing engraved sound tracks, said record comprising a tanned colloid and the light decomposition product of a light-sensitive dyestuff.

50

12. A phonograph record bearing engraved sound tracks, said record comprising a tanned colloid and the light decomposition product of a light-sensitive xanthone dyestuff.

55

13. A phonograph record bearing engraved sound tracks, said record comprising a tanned colloid and the light decomposition product of a high molecular diazo compound which contains at least three carbocyclic rings.

60

14. A phonograph record bearing engraved sound tracks, said record comprising a tanned colloid and the light decomposition product of a light-sensitive nitro compound.

65

15. A phonograph record bearing engraved sound tracks, said record comprising a tanned colloid and the light decomposition product of an alpha-nitro-naphthalene sulfonic acid.

70

GUSTAV KÖGEL.